

## UNITED STATES PATENT OFFICE

SAMUEL H. HARTMAN AND HENRY L. POWERS, OF LANCASTER, PENNSYLVANIA, AS  
SIGNORS TO ARMSTRONG CORK COMPANY, OF LANCASTER, PENNSYLVANIA, A COR-  
PORATION OF PENNSYLVANIA

## GREENS MATERIAL

No Drawing.

Application filed September 19, 1930. Serial No. 483,130.

This invention relates to a greens material such as may be employed, for example, in the surfacing of miniature golf courses, although it has numerous other applications. 5 It may be employed as a greens material on full-sized golf courses where it is difficult, because of climatic conditions, to maintain grass greens, or around the base of Christmas trees. It will hereinafter be particularly described as applied to miniature golf courses.

Golf courses of this character are usually constructed of a surface material laid over a porous bed. Various materials have been 15 proposed for surfacing:—for example, materials consisting essentially of cottonseed hulls, chicken feathers, peat moss, sawdust, sand, etc. Numerous objections have been raised to all of these materials. Some of 20 them tend to pack too hard or to scuff up unduly under traffic. They may require a large amount of raking, rolling or sprinkling. They may absorb such a large quantity of moisture as to require the loss of a 25 great deal of time after a rain, or they may stain the shoes of players or be of such character that they do not adapt themselves readily to contouring over hazards and obstacles in the course.

30 We have found a composition which overcomes all of these defects and provides a peculiarly desirable playing surface. We employ a material consisting essentially of saturated fibrous material. More specifically, 35 we may employ comminuted felt-base scrap. Felt-base floor coverings are well known and a material amount of scrap is produced during manufacture. This material consists of a web of felt saturated with a bituminous material. We find that by grinding the same it 40 forms the basis of a very desirable greens material. While a considerable amount of pigment is required in order to give it the proper color, the particles are inherently of such character as to be reasonably coherent. Consequently, on tamping or rolling the material compacts in a sufficient amount to serve 45 the purpose, although it never packs to such a point as to permanently unite the particles. We preferably employ with this ma-

terial a bulking filler or fillers, and also incorporate a suitable oil in the mix. A preferred composition is as follows:

|                                      |            |    |
|--------------------------------------|------------|----|
| Ground-up felt base                  | 200 pounds | 55 |
| Wood flour                           | 50 pounds  |    |
| Sand or other inert bulking material | 90 pounds  |    |
| Paraffin oil                         | 10 gallons |    |

To the above is added a mineral pigment 60 in the amount of approximately 5 pounds for each 100 pounds of the mix. The dry constituents are first mixed together, as, for example, in an ordinary concrete mixer, and then the oil is added, the mixing being continued until thorough distribution has been obtained.

Various bulking fillers, such as slate flour, powdered limestone, kaolin, or the like may 70 be substituted wholly or in part for the sand. Other oils, such as creosote oils, may be employed. We prefer that the oil shall be of a non-drying character so that the qualities of the composition are indefinitely retained. The pigment is preferably a mineral pigment 75 in powdered form. This is preferable to a dye or stain, because the latter tend to fade out, thus giving a non-uniform color if a green has been patched or repaired.

Our material is very resistant to scuffing 80 and has excellent qualities of resilience. It is not adversely affected by rain and can be played on within a few minutes after a thorough wetting. The surface is about equivalent to grass so far as the speed of the ball is concerned. The material does not pack 85 down and lie dead, although the character of the playing surface can be adjusted over a wide range by rolling if it is desired to make the course faster, or by light raking or wetting if a slower course is wanted.

A great advantage of our invention is that 90 it provides an outlet for waste materials. Felt base and roofing are two examples of materials whose scrap may be readily employed. There are numerous other industries, however, in which saturated fibrous material is employed, and the scrap therefrom finds ready disposal in accordance with the present invention.

We have given a preferred embodiment of our invention by way of example only. It will be understood that it is not thus limited but may be otherwise embodied within the scope of the following claims.

We claim:

1. A surfacing material for golf greens comprising comminuted saturated fibrous material which is inherently coherent but not permanently united, said surfacing material being relatively loose, porous, waterproof, resilient and resistant to scuffing.
  2. A surfacing material for golf greens comprising comminuted saturated fibrous material which is inherently coherent but not permanently united and an inert bulking filler, said surfacing material being relatively loose, porous, waterproof, resilient and resistant to scuffing.
  3. A surfacing material for golf greens comprising villous comminuted saturated fibrous material which is inherently coherent but not permanently united, an inert bulking filler and a nondrying oil, said surfacing material being relatively loose, porous, waterproof, resilient and presenting a surface simulating the texture of natural grass.
  4. A surfacing material for golf greens comprising comminuted bitumen-saturated fibrous material which is inherently coherent but not permanently united, sand, a mineral pigment and paraffin oil, said surfacing material being relatively loose, porous, waterproof, resilient, resistant to scuffing and presenting a surface simulating the texture of natural grass.
  5. A surfacing material for golf greens comprising substantially 200 parts of comminuted bitumen-saturated fibrous material which is inherently coherent but not permanently united, 90 parts of sand and 10 parts of paraffin oil, said surfacing material being relatively loose, porous, waterproof, resilient and resistant to scuffing.
- 45 In testimony whereof we have hereunto set our hands.

SAMUEL H. HARTMAN.

HENRY L. POWERS.